

April 7, 1925.

1,532,113

N. AHLMANN

## PROCESS OF AGGLOMERATING ORE AND THE LIKE

Filed Oct. 20, 1922

2 Sheets-Sheet 1

Fig. 1.



Fig. 2.



*INVENTOR*

Nikolai Ahlmann  
BY  
Redding & Hesley, ATTORNEY

*ATTORNEYS*

April 7, 1925.

1,532,113

N. AHLMANN

PROCESS OF AGGLOMERATING ORE AND THE LIKE

Filed Oct. 20, 1922

2 Sheets-Sheet 2

*Fig 3.*



INVENTOR

*Nikolai Ahlmann*

BY

*Redding Greely*

ATTORNEYS

Patented Apr. 7, 1925.

1,532,113

# UNITED STATES PATENT OFFICE.

NIKOLAI AHLmann, OF COPENHAGEN, DENMARK.

## PROCESS OF AGGLOMERATING ORE AND THE LIKE.

Application filed October 20, 1922. Serial No. 595,858.

To all whom it may concern:

Be it known that I, NIKOLAI AHLmann, a subject of the King of Denmark, residing at 22 F. Hørsholmsgade, Copenhagen, Denmark, have invented certain new and useful Improvements in Processes of Agglomerating Ore and the like, of which the following is a specification.

In the agglomeration of pulverous ore in rotary kiln it is as a rule necessary, in order to obtain an agglomerate with a small proportion of dust, to heat the ore to such a high degree that sintering, i. e. a partial melting of the material, takes place in the kiln. The resulting agglomerate will then consist of lumps, or so-called nodules, which are often of sufficient mechanical strength and at the same time somewhat porous, but do not possess the high degree of porosity which is required for the subsequent treatment of the nodules in blast furnaces. On the other hand, a high degree of porosity can be attained at the sacrifice of the mechanical strength by briquetting the pulverous ore in a cold state and burning the resulting briquettes at such low temperature that no sintering will be created.

It is, however, known that for the melting of the ore in blast furnaces the nodules should combine a high degree of porosity with great mechanical strength, and it is the purpose of the present invention to attain this result.

The invention is based upon the discovery that at a temperature materially lower than the sintering temperature the pulverous ore will be of such consistency that by pressure the grains of the ore can be made to stick strongly together while at the same time the mass of material will have a very high porosity.

In accordance with the invention, therefore, the pulverous ore is heated in a rotary kiln to the temperature required which, as it will be understood, is lower than the sintering temperature for the ore, and then, while it has still this temperature, is pressed, in a suitable machine, either into briquettes or into other suitable form.

50 In the accompanying drawing—

Figure 1 is a partial view, in vertical section and in outline, of apparatus in which the invention can be practiced.

55 Figure 2 is a plan view in outline of the press shown in Figure 1.

Figure 3 is a view similar to Figure 1 but showing a different form of press.

The particular design of apparatus employed in the practice of the invention is unimportant, but it should be constructed with due regard to the fact that it has to treat glowing material. In Figures 1 and 2 of the drawing is illustrated somewhat diagrammatically a form of apparatus adapted for the practice of the invention, comprising a rotary kiln *a* with a hood *b* and a suitable fuel nozzle *c* by which the flame is directed as usual into the kiln. From the kiln the hot material may fall into a hopper *d* from which it is delivered to a rotating table *e* which is provided with molds *f* lined with fire brick *g*. As the table *e*, supported upon a suitable base *h*, is rotated with a step by step motion the heated material in each mold, at a point opposite the hopper *d*, is subjected to the pressure of a suitable plunger *i* and the briquette thus formed is discharged in the further movement of the press table *e*, through an opening provided at *k* in the base *h*.

In the form of apparatus shown in Figure 3 the kiln *a*, hood *b*, fuel nozzle *c* and hopper *d* are arranged substantially as shown in Figure 1. From the hopper *d* the heated material is delivered into a water cooled cylinder *l* and is there subjected to pressure between two pistons *m*, *n*, the piston *m* being then withdrawn to permit the discharge of the briquette by the continued forward movement of the piston *n*.

Other forms of apparatus in which the invention can be practiced will suggest themselves. It will be obvious, for example, that the heating of the pulverous ore to the temperature suitable for the briquetting might be effected by the rapid oxidation brought about by forcing a current of air or of a mixture of air and water vapor through the pulverous ore which has been heated and more or less reduced in the kiln.

I claim as my invention:

The process of agglomerating pulverous ore which consists in heating the pulverous material to a temperature less than the sintering temperature and then subjecting the heated material to pressure to form a coherent, porous mass.

This specification signed this 5th day of October, A. D. 1922.

NIKOLAI AHLmann.